# EUROPEAN PATENT SPECIFICATION

(11) **EP 3 161 174 B1**
(45) Date of publication and mention of the grant of the patent: **06.06.2018**
(21) Application number: 15733673.6
(22) Date of filing: 25.06.2015
(51) Int. Cl.: C22C 19/05, C22C 38/00, C22C 38/02, C22C 38/04, C22C 38/06, C22C 38/42, C22C 38/44, C22C 38/48, C22C 38/50, C22C 38/52, F04D 29/02, B22F 5/00, C21D 6/00, C22C 33/02

(54) **COMPONENT OF A TURBOMACHINE, TURBOMACHINE AND PROCESS FOR MAKING THE SAME**
KOMPONENTE EINER TURBOMASCHINE, TURBOMASCHINE UND VERFAHREN ZUR HERSTELLUNG DAVON
ÉLÉMENT CONSTITUTIF D'UNE TURBOMACHINE, TURBOMACHINE ET LEUR PROCÉDÉ DE FABRICATION

(30) Priority: 27.06.2014 IT CO20140021
(43) Date of publication of application: 03.05.2017
(73) Proprietor: Nuovo Pignone S.r.l., 50127 Florence (IT)
(72) Inventor: CAPPUCCINI, Filippo, 50127 Florence (IT); ROMANELLI, Marco, 50127 Florence (IT); DI PIETRO, Domenico, 50127 Florence (IT); BUCCIONI, Massimiliano, 50127 Florence (IT); PIETRANGELI, Emanuele, 50127 Florence (IT)
(74) Representative: Illingworth-Law, William Illingworth
(86) International application number: PCT/EP2015/064350
(87) International publication number: WO 2015/197751

(56) References cited:
- EP-A1- 0 052 941
- EP-A1- 0 136 998
- WO-A1-2006/111520
- JP-A- S61 163 238
- US-A- 4 818 483
- US-A- 5 378 427
- US-A- 5 945 067
- TSAPRAILIS AND L F GARFIAS-MESIAS H: "Rapid Evaluation of Metallic Coatings on Large Cylinders Exposed to Marine Environments", CORROSION, NACE INTERNATIONAL, HOUSTON, TX; US, US, vol. 67, no. 12, December 2011 (2011-12), pages 126002-1, XP001570961, ISSN: 0010-9312, DOI: 10.5006/1.3666861

## Description

### FIELD

Embodiments of the subject matter disclosed herein relate in general to components for turbomachines and to turbomachines for "Oil & Gas" applications.

Some embodiments relate to (rotary) centrifugal compressors or pumps, as well as their components, operating in the field of production and treatment of oil and gas containing e.g. hydrocarbon plus hydrogen sulfide, carbon dioxide, with or without other contaminants. These materials are referred as "sour gas". Such apparatuses have at least one component made of a high corrosion resistant alloy, capable of resisting to corrosion better than state of art martensitic stainless steels and behaving similarly to premium nickel base superalloys.

Some embodiments relate to (rotary) gas turbines or steam turbines, as well as their components. Such apparatuses have at least one component made of a high mechanical resistant alloy, capable of resisting to fatigue and/or creep better than state of art materials.

### BACKGROUND ART

A compressor is a machine capable of raising the pressure of a compressible fluid (gas) through the use of mechanical energy. In centrifugal compressors, the compression of the fluid is carried out by one or more impellers assembled on a shaft with a rotating motion inside one or more stator parts (diaphragm) stacked together by bolts. The described assembly is normally called bundle. The fluid to be compressed is drawn into the bundle through one or more intake ducts, whereas the compressed fluid is expelled from the bundle towards one or more delivery ducts.

Commonly, the centrifugal compressors are actuated by electric motors or else by internal combustion engines, through a coupling for transmitting the motion.

Centrifugal compressors that operate in sour gas fields are subject to different type of interaction with the environment (corrosion) that can cause loss of performance and premature failure of compressor components.

The sour service is characterized by hydrocarbons with wet hydrogen sulphide (H₂S) where the pH₂S is higher than 0.0030 bar. This value is valid for carbon and low alloy steels. NACE MR0175/ISO 15156-1 doesn't define a minimum pH₂S limit for corrosion resistant alloys (CRAs), because this limit is a function also of acidity of the solution (pH) and the values can be lower than the one defined for carbon and low alloy steels.

There are several corrosion phenomena, where the following types are the most relevant:
- General corrosion - an even attack of the surface of the material
- Pitting corrosion - an uneven localized attack
- Stress corrosion cracking (SCC and CSCC)

It is pointed out that corrosion phenomena listed above can only occur if condensed water is present (wet gas), that acts as electrolyte for electrochemical process.

Wet gas containing hydrocarbons, CO₂, H₂S, and chlorides (or other halides) eventually in presence of elemental sulphur, represents an environment where all the phenomena listed above can occur.

Resistance of material to single or combination of damage mechanisms is therefore fundamental in order to guarantee reliability of products.

Among the corrosion mechanism listed above, the most critical is the stress corrosion cracking either by wet H₂S or chlorides (or in general halides), because it makes unavailable the unit for service.

In general, the mechanism involves the diffusion in the metal of hydrogen atoms generated by corrosion.

SSC can occur only if the following three conditions are verified:
- Tensile stress (residual and/or applied)
- H₂S + condensed water
- Material prone to SSC damage

Contaminants such as halides, arsenic (As), antimony (Sb) and cyanides (CN⁻) act as catalyst, increasing the concentration of hydrogen atoms on surface and by preventing their recombination in hydrogen molecules making SSC more severe.

In general, centrifugal compressor components (impellers, shafts, diaphragms and bolts) are exposed to tensile stress and wet gas conditions.

Based upon experience, it has been found that the impellers and bolts constitute the most prone components to SSC and CSCC. This because the stress level is higher than in the other components and because the stress remains applied during compressor stops (pressurized) where a wet gas at higher partial pressure occurs. Therefore is mandatory, for sour service environments, to select materials that are able to withstand the severe environment conditions.

Material selection for such service is therefore based on a three dimensional space governed by partial pressure of H₂S (p(H₂S)), pH (mainly function of CO₂), and chlorides (and/or other halides) content, as schematically represented in Figure 1.

Up to now different materials have been used with the aim of selecting the most cost effective solution for the specified environment.

In order to simplify the complex rules behind material fit for purpose approach, the following principles cloud be considered:
- For low p(H₂S) any pH, and high chlorides content duplex and superduplex alloys are the class of material of choice;
- For low to moderate p(H₂S), any pH and low chlorides different classes of martensitic stainless steels are the class of material of choice;
- For any p(H₂S), any pH and high chlorides nickel based alloys are the class of material of choice;

Representing these principles above in the 3D space, it is clear that there is a huge space between cost effective alloys (i.e. duplex, superduplex and martensitic stainless steels) and premium nickel base alloys, that could be covered by new alloys.

Therefore, there is a need for components for centrifugal compressors in particular, but not exclusively on compressors operating in the field of production and treatment of oil and gas containing hydrocarbon plus hydrogen sulfide with or without other contaminants, capable of improving the reliability, increase the speed (given the higher specific strength of material) and provide a cost effective alloy by reducing expensive alloying elements, mainly nickel.

Similar problems need to be addressed in pump design and service conditions or in some steam turbine application (i.e. geothermal fields).

A gas turbine is a type of internal combustion engine. It has an upstream rotating compressor coupled to a downstream turbine, and a combustion chamber in-between.

Atmospheric air flows through a compressor is brought to higher pressure in a combustion chamber where it is mixed and burnt with fuel (i.e liquid or gas) to increase its enthalpy. This high-temperature highpressure flow enters in an expansion turbine, producing a shaft work output in the process. The turbine shaft work is used to drive the compressor and other devices such as an electric generator that may be coupled to the shaft.

This environment is characterized by a combination of high temperature, high stress in steady and cycling conditions. Materials for such application shall be designed to withstand creep, low and high cycle fatigue, oxidation and corrosion. This is normally accomplished by high strength steels or nickel base alloys.

Similar problems need to be addressed in steam turbine design and service conditions.

The present Inventors have tried to achieve one or some or all of the above objects.

TSAPRAILIS AND L F GARFIAS-MESIAS H: "Rapid Evaluation of Metallic Coatings on Large Cylinders Exposed to Marine Environments", CORROSION, NACE INTERNATIONAL, HOUSTON, TX; US, US, vol. 67, no. 12, December 2011 (2011-12), pages 126002-1, discloses the corrosion resistant alloys such as UNS N09925 alloys, suitable for the fabrication of hydraulic cylinders and piston rods.

### SUMMARY

According to first exemplary embodiments, there is a component of a turbomachine, the component being made of an alloy having a chemical composition consisting of:

| | |
|---|---|
| C | 0.005-0.03 wt% |
| Si | 0.05-0.5 wt% |
| Mn | 0.1-1.0 wt% |
| Cr | 19.5-22.5 wt% |
| Ni | 35.0-37.0 wt% |
| Mo | 3.0-5.0 wt% |
| Cu | 1.0-2.0 wt% |
| Co | 0.0-1.0 wt% |
| Al | 0.01-0.5 wt% |
| Ti | 1.8-2.5 wt% |
| Nb | 0.2-1.0 wt% |
| W | 0.0-1.0 wt% |

based on the alloy weight, the remaining being Fe and impurities, said impurities comprising S 0.0-0.01 wt% and P 0.0-0.025 wt%.

According to second exemplary embodiments, there is a process for making the above component, said process comprising at least one of the following steps of:
a) melting the chemical composition of claim 1 through vacuum induction melting (VIM), or arc electric furnace;
b) refining by Argon Oxygen Decarburization (A.O.D.), Vacuum Induction Degassing and Pouring (V.I.D.P), or Vacuum Oxygen Decarburization (V.O.D.);
c) re-melting through electro-slag re-melting (E.S.R.), or vacuum arc re-melting (VAR).

According to third exemplary embodiments, there is a turbomachine comprising at least one component as defined in general above.

### BRIEF DESCRIPTION OF THE DRAWINGS

The present invention will become more apparent from the following description of exemplary embodiments to be considered in conjunction with accompanying drawings wherein:
Figure 1 shows a three dimensional space governed by partial pressure of H₂S (p(H₂S)), pH (mainly function of CO₂), and chlorides (and/or other halides) content;
Figure 2 shows a typical cross section of centrifugal compressor;
Figure 3 shows a typical cross section of centrifugal pump;
Figure 4 shows a typical cross section of a steam turbine;
Figure 5 shows a typical cross section of a gas turbine;
Figure 6A shows the phase equilibrium vs temperature of the alloy of Example 1 and Figure 6B shows the phase equilibrium vs temperature of the comparative UNS N07718; and
Figure 7A shows the Time Temperature Transformation curves for the alloy of Example 1 and Figure 7B shows the Time Temperature Transformation curves for the comparative UNS N07718.

### DESCRIPTION

The following description of exemplary embodiments refer to the accompanying drawings. The same reference numbers in different drawings identify the same or similar elements. The following detailed description does not limit the invention. Instead, the scope of the invention is defined by the appended claims.

Reference throughout the specification to "one embodiment" or "an embodiment" means that a particular feature, structure, or characteristic described in connection with an embodiment is included in at least one embodiment of the subject matter disclosed. Thus, the appearance of the phrases "in one embodiment" or "in an embodiment" in various places throughout the specification is not necessarily referring to the same embodiment. Further, the particular features, structures or characteristics may be combined in any suitable manner in one or more embodiments.

The term "room temperature" as used herein has its ordinary meaning as known to those skilled in the art and may include temperatures within the range of about 16°C (60°F) to about 32°C (90°F).

Regarding the alloy composition, the term "mandatory element" refers to an element that is present in the alloy and that, in combination with the other mandatory elements, allows to achieve the above objects. The mandatory elements in the alloy are Iron (Fe), Carbon (C), Silicon (Si), Manganese (Mn), Chromium (Cr), Nickel (Ni), Molybdenum (Mo), Copper (Cu), Aluminium (Al), Titanium (Ti), and Niobium (Nb).

The term "optional element" refers to an element that is possibly present in addition to the mandatory elements defining the essential chemical composition of the alloy. The optional elements in the alloy are: Cobalt (Co), and Tungsten (W).

The term "impurity" or "impurity element", instead, refers to an element not provided in the design of the alloy composition in order to reach the aforesaid objects. However, said element may be present because, depending on the manufacturing process, its presence may be unavoidable. Impurities in the alloy comprise phosphorous (P), Sulphur (S), Boron (B), Bismuth (Bi), Calcium (Ca), Magnesium (Mg), Silver (Ag), Lead (Pb), Nitrogen (N), Tin (Sn), and Oxygen (O).

In one embodiment, at least one component of a turbomachine is made of a high corrosion high temperature resistant alloy, capable of resisting to corrosion and/or stress at high temperature better than state of art martensitic stainless steels and behaving similarly to premium nickel base superalloys like those complying the requirements of UNS N07718 e UNS N00625. Said alloy has a chemical composition consisting of:

| | |
|---|---|
| C | 0.005-0.03 wt% |
| Si | 0.05-0.5 wt% |
| Mn | 0.1-1.0 wt% |
| Cr | 19.5-22.5 wt% |
| Ni | 35.0-37.0 wt% |
| Mo | 3.0-5.0 wt% |
| Cu | 1.0-2.0 wt% |
| Co | 0.0-1.0 wt% |
| Al | 0.01-0.5 wt% |
| Ti | 1.8-2.5 wt% |
| Nb | 0.2-1.0 wt% |
| W | 0.0-1.0 wt% |

based on the alloy weight, the remaining being Fe and impurities, said impurities comprising S 0.0-0.01 wt% and P 0.0-0.025 wt%.

The above alloy is advantageously a cost effective alloy, which at the same time surprisingly encompasses a reduced amount of expensive alloying elements, such as mainly nickel, but also chromium, molybdenum and titanium, without negatively affecting the mechanical and anticorrosion properties. Said alloy also shows a great resistance to high temperatures and pressures, so that the components made of the same result to be advantageously suitable for turbomachines, particularly centrifugal compressors.

Said impurities are P, S, B, Bi, Ca, Mg, Ag, Pb, N, Sn, O or a combination thereof.

Preferably, said impurities are less than 0.5 wt%; more preferably, less than 0.2 wt%.

In preferred embodiments, said impurities are P up to 0.025 wt%, S up to 0.01 wt%, B, Bi, Ca, Mg, Ag, Pb, N, Sn, and O.

In some embodiments, the alloy has high resistance to corrosion at high temperature, in particular in the range of 200-250°C.

In other embodiments, the alloy has high resistance to fatigue and/or creep at high temperature, in particular in the range of 400-700°C.

In preferred embodiments, the alloy has a chemical composition consisting of:

| | |
|---|---|
| C | 0.005-0.03 wt% |
| Si | 0.05-0.2 wt% |
| Mn | 0.1-0.6 wt% |
| Cr | 20.0-21.5 wt% |
| Ni | 35.0-37.0 wt% |
| Mo | 3.5-4.0 wt% |
| Cu | 1.2-2.0 wt% |
| Co | 0.0-0.2 wt% |
| Al | 0.05-0.4 wt% |
| Ti | 1.9-2.3 wt% |
| Nb | 0.2-0.5 wt% |
| W | 0.0-0.6 wt% |

based on the alloy weight, the remaining being Fe, with Fe at least 30 wt%, and impurities, said impurities comprising S 0.0-0.001 wt% and P 0.0-0.02 wt%.

In more preferred embodiments, the alloy has a chemical composition consisting of:

| | |
|---|---|
| C | 0.005-0.02 wt% |
| Si | 0.05-0.2 wt% |
| Mn | 0.1-0.6 wt% |
| Cr | 20.0-21.5 wt% |
| Ni | 35.0-37.0 wt% |
| Mo | 3.5-4.0 wt% |
| Cu | 1.2-2.0 wt% |
| Co | 0.0-0.2 wt% |
| Al | 0.05-0.4 wt% |
| Ti | 1.9-2.3 wt% |
| Nb | 0.2-0.5 wt% |
| W | 0.0-0.6 wt% |

based on the alloy weight, the remaining being Fe, with Fe at least 30 wt%, and impurities, said impurities comprising S 0.0-0.001 wt% and P 0.0-0.02 wt%.

In even more preferred embodiments, the alloy has a chemical composition consisting of:

| | |
|---|---|
| C | 0.005-0.02 wt% |
| Si | 0.06-0.15 wt% |
| Mn | 0.2-0.4 wt% |
| Cr | 20.2-21.0 wt% |
| Ni | 36.0-36.5 wt% |
| Mo | 3.6-3.8 wt% |
| Cu | 1.3-1.7 wt% |
| Co | 0.0-0.1 wt% |
| Al | 0.1-0.3 wt% |
| Ti | 2.0-2.2 wt% |
| Nb | 0.25-0.4 wt% |
| W | 0.0-0.4 wt% |

based on the alloy weight, the remaining being Fe, with Fe at least 30 wt%, and impurities, said impurities comprising S 0.0-0.001 wt% and P 0.0-0.015 wt%.

In the most preferred embodiments, the alloy has a chemical composition consisting of:

| | |
|---|---|
| C | 0.015 wt% |
| Si | 0.09 wt% |
| Mn | 0.3 wt% |
| Cr | 20.4 wt% |
| Ni | 36.2 wt% |
| Mo | 3.7 wt% |
| Cu | 1.41 wt% |
| Co | 0.03 wt% |
| Al | 0.25 wt% |
| Ti | 2.04 wt% |
| Nb | 0.27 wt% |
| W | 0.1 wt% |
| Fe | balance |

having the following impurities:

| | |
|---|---|
| P | up to 0.013 wt% |
| S | up to 0.0002 wt% |
| B | up to 0.003 wt% |
| Bi | up to 0.3 ppm |
| Ca | up to 50 ppm |
| Mg | up to 30 ppm |
| Ag | up to 5 ppm |
| Pb | up to 5 ppm |
| N | up to 100 ppm |
| Sn | up to 50 ppm |
| O | up to 50 ppm |

In some embodiments, the alloy has a grain size finer than plate 3 as per ASTM E112.

The above alloy can be obtained by any casting process. However, it is preferred to obtain said alloy by a process comprising at least one of the following steps of:
a) melting the above chemical composition through vacuum induction melting (VIM), or arc electric furnace;
b) refining by Argon Oxygen Decarburization (A.O.D.), Vacuum Induction Degassing and Pouring (V.I.D.P), or Vacuum Oxygen Decarburization (V.O.D.);
c) re-melting through electro-slag re-melting (E.S.R.), or vacuum arc re-melting (VAR).

In this way, the presence of impurities, segregation thereof and in-homogeneities is significantly reduced and at the same time improved mechanical characteristics and corrosion resistance of the alloy are achieved.

In some embodiments, the alloy resulting from the above described casting processes is subjected to a step d) of homogenization at a high temperature, preferably above 1100° C for at least 6 hours.

In some embodiments, the alloy resulting from the above described casting processes and subsequent step d) of homogenization heat treatment, is further subjected to a step e) of hot or cold plastic deformation through at least one plastic deformation cycle, in order to attain a minimum total reduction ratio of 2:1. Such plastic deformation cycles include forging (open or close die), rolling, extrusion, cold expansion, to produce a raw component shape or more generally a raw shape to be further machined to produce centrifugal compressor, pump, gas and steam turbine, as well as components thereof.

In other embodiments, the alloy resulting from step e) is then subjected to a step f) of heat treatment to induce solubilization through at least one heat cycle, preferably at a temperature of 1020-1150°C, that can be carried out inside furnaces, under air, controlled atmosphere or vacuum, and followed by fast cooling in liquid or gas media, in order to put and keep in solution the alloying elements (i.e copper, titanium, aluminium, niobium, etc...) for optional subsequent heat treatment steps.

In further embodiments, said step f) of heat treatment is followed by a step g) of an ageing treatment.

Preferably, said step g) of an ageing treatment comprises the following sub-steps:
g-1) heating the alloy to a temperature of 710-780°C for 4-8 h;
g-2) cooling at a cooling rate of 40-60°C/h down to a temperature of 610-670°C;
g-3) keeping the alloy to a temperature of 610-670°C for at least 6 h, and
g-4) letting the alloy to cool at room temperature in air.

Alternatively, said step g) of an ageing treatment comprises the following sub-steps:
g-1') heating the alloy to a temperature of 780-820°C for 2-8 h; and
g-2') letting the alloy to cool at room temperature in air.

Owing to the above described chemical composition, level of impurities, grain size resulting from controlled plastic deformation process and heat treatment conditions, the alloy advantageously shows the following properties:
- superior anticorrosion characteristics in terms of general and localized corrosion, threshold stress in solution A method A as per NACE MR0175, higher Stress Corrosion Cracking (SCC) resistance, higher Chloride Stress Corrosion Cracking (CSCC), Sulphide Stress Cracking (SSC), Galvanically-induced Hydrogen Stress Cracking (GHSC);
- higher tensile properties at room and high temperature;
- suitable toughness properties;
- higher high and low cycle fatigue properties;
- higher creep strength;
- higher oxidation and hot corrosion resistance;
with respect to stainless steels (martensitic, ferritic, austenitic and austenitic-ferritic) and comparable to premium nickel base superalloys.

In some embodiments, the alloy is further atomized to produce powder and then treated by powder metallurgy. Preferably, with the term "powder metallurgy" it is meant that said powder is consolidated by Cold Isostatic Pressing (CIP), by Metal Injection Moulding (MIM), Sintering, Hot Isostatic Pressing (HIP), or fabricated by MIM and exposed to a HIP process. Basically, powders are fed into a die, compacted to a desired shape. The pressed powder is then sintered or hipped in a controlled atmosphere furnace at room or high pressure to produce metallurgical bonds among powder particles. Optional post-sintering operations, such as isothermal forging, infiltration, finish machining or surface treatment, may then be applied to complete the component.

Figures 2, 3, 4 and 5 show different turbomachines where one or more components as set out above may be used. Figure 2 shows a typical cross section of centrifugal compressor, Figure 3 shows a typical cross section of centrifugal pump, Figure 4 shows a typical cross section of a steam turbine, and Figure 5 shows a typical cross section of a gas turbine.

Thanks to its high resistance to corrosion (even at high temperature) and/or to its high resistance to fatigue and/or creep, the component is very useful, in particular it is very useful for components that get in touch with the working fluid of the turbomachine.

### EXAMPLES

### Example 1.

An alloy has been prepared having the following composition:

| | |
|---|---|
| C | 0.015 wt% |
| Si | 0.09 wt% |
| Mn | 0.3 wt% |
| Cr | 20.4 wt% |
| Ni | 36.2 wt% |
| Mo | 3.7 wt% |
| Cu | 1.41 wt% |
| Co | 0.03 wt% |
| Al | 0.25 wt% |
| Ti | 2.04 wt% |
| Nb | 0.27 wt% |
| W | 0.1 wt% |
| Fe | balance |

having the following impurities:

| | |
|---|---|
| P | up to 0.013 wt% |
| S | up to 0.0002 wt% |
| B | up to 0.003 wt% |
| Bi | up to 0.3 ppm |
| Ca | up to 50 ppm |
| Mg | up to 30 ppm |
| Ag | up to 5 ppm |
| Pb | up to 5 ppm |
| N | up to 100 ppm |
| Sn | up to 50 ppm |
| O | up to 50 ppm |

The above chemical composition was melted through vacuum induction melting (VIM), refined by Argon Oxygen Decarburization (A.O.D.), and re-melted re-melting through electro-slag re-melting (E.S.R.).

The resulting alloy was homogenized at a temperature above 1100° C for at least 6 hours.

The alloy was then subjected to two cycles of hot plastic deformation.

Subsequently, the alloy was subjected to a heat treatment to induce solubilization at a temperature of 1020-1150°C, followed by fast cooling in liquid or gas media.

The resulting alloy has been tested to assess mechanical and anticorrosion properties. The results have been compared to a known Martensitic Stainless Steel (shortly 'Martensitic SS') in the following Table 1.

Martensitic Stainless steels is a category of stainless steels having a microstructure mainly composed by tempered Martensite. Matertensite is formed by a rapid cooling of austenite phase which is achieved by a quenching heat treatment. Traditional martensitic steels have a high carbon content, in the 0.08-1.% range, a Chromium in the 12-17% range. Their main characteristic compared other stainless steel classes is the high strength and fair corrosion resistance.

**Table 1.**

| **Corrosion Characteristic** | **Typical Martensitic SS** | **Alloy of Example 1** |
|---|---|---|
| Critical Pitting Temperature (CPT)AST G48 method C [°C] | 0÷5°C | 30÷40°C |
| Sulfide Stress Corrosion (SSC) Threshold in NACE TM0177 Solution A method A [MPa] | 250÷300 MPa (<50%AYS) | 750÷800 Mpa (>95%AYS) |
| Chloride Stress Corrosion Cracking ASTM G123 | Failure <300h | Passed ≥1000h |

Additional verified SSC properties are reported in Table 2 and Table 3.

**Table 2.**

| | Method | pH₂S | pH | Chlorides | Stress | Temperature | Result |
|---|---|---|---|---|---|---|---|
| **Alloy of Example 1** | NACE TM0177 Method A Solution C | 10 bar | 3 | 25%NaCl | 750MPa | 25°C | Passed (>720h) |
| | | 10 bar | 3 | 25%NaCl | 750MPa | 150°C | Passed (>720h) |

**Table 3.**

| **Characteristics** | **High Temperature Martensitic SS** | **Alloy of Example 1** |
|---|---|---|
| Stress Rupture | 600°C, 240Mpa, 140hrs | 600°C, 690Mpa, 140hrs |
| Tensile @600°C | 430MPa | 550Mpa |
| Impact Charpy -V notch | 27J @-15°C | 27J @-101°C |

The alloying elements' weight percent is tailored to avoid or minimizing topologically closed packed phases (TCP). Excessive quantities of Cr, Mo, W would promote the precipitation of intermetallic phases which are rich in these elements. Generally speaking, the TCP phases have chemical formulae AₓB_{y}. For example, the µ phase is based on the ideal stoichiometry A₆B₇ and has a rhombohedral cell containing 13 atoms, such as W₆Co₇ and Mo₆Co₇.

The σ phase is based upon the stoichiometry A₂B and has a tetragonal cell containing 30 atoms, such as Cr₂Ru, Cr₆₁Co₃₉ and Re₆₇Mo₃₃.

The P phase, for example, Cr₁₈Mo₄₂Ni₄₀ is primitive orthorhombic, containing 56 atoms per cell.

As it is shown in Figures 6A (thermodynamic equilibrium) and 7A (kinetics estimation), only σ phase is thermodynamically possible and precipitation kinetics is so slow that neither during solution annealing, nor during ageing can happen.

The chemical composition of this alloy is optimized to enlarge the hot workability window. This is accomplished by a low nickel content and reducing the temperature of precipitation of hardening secondary phases (gamma prime). As it can be seen in Figure 6, the theoretic workability range at equilibrium is quite large and is between 1020°C and 1280°C. This interval is larger than those provided by UNS N07718 (Figures 6B and 7B).

Equilibrium intervals do not take into account kinetics and visco-plastic phenomena, but can give an idea of how much better this alloy behaves in comparison with other well known commercial premium nickel base alloys.

Practically, this alloy has a hot forming range between 900°-1200°C, thus reducing the risk of failure during production and cycle time.

The alloy has a combination of chemical elements so as to provide secondary phases hardening such as to provide a minimum yield strength of 750 Mpa with a max hardness of 34 HRC thus enhancing stress corrosion properties.

The reduced hardness level results in a better machining if compared with premium nickel based alloys like UNS N07718. This level of hardness allows the turbomachinery components to be machined in aged conditions resulting in an optimization of manufacturing cycle if compared with premium nickel based alloys like UNS N07718.

This alloy is designed to be easy welded by common arc welding processes (SMAW and GTAW) with homologous or different nickel base filler materials like UNS N06625, UNS N07725, or UNS N09925.

## Claims

1. A component of a turbomachine, the component being made of an alloy having a chemical composition consisting of:
| | |
|---|---|
| C | 0.005-0.03 wt% |
| Si | 0.05-0.5 wt% |
| Mn | 0.1-1.0 wt% |
| Cr | 19.5-22.5 wt% |
| Ni | 35.0-37.0 wt% |
| Mo | 3.0-5.0 wt% |
| Cu | 1.0-2.0 wt% |
| Co | 0.0-1.0 wt% |
| Al | 0.01-0.5 wt% |
| Ti | 1.8-2.5 wt% |
| Nb | 0.2-1.0 wt% |
| W | 0.0-1.0 wt% |
based on the alloy weight, the remaining being Fe and impurities, said impurities comprising S 0.0-0.01 wt% and P 0.0-0.025 wt%.

2. The component of claim 1, wherein the alloy has a high resistance to corrosion at a high temperature, in particular in the range of 200-250°C.

3. The component of claim 1 or 2, wherein the alloy has a high resistance to fatigue and/or creep at a high temperature, in particular in the range of 400-700°C.

4. The component of any one of claims 1-3, wherein the alloy has a chemical composition consisting of:
| | |
|---|---|
| C | 0.005-0.03 wt% |
| Si | 0.05-0.2 wt% |
| Mn | 0.1-0.6 wt% |
| Cr | 20.0-21.5 wt% |
| Ni | 35.0-37.0 wt% |
| Mo | 3.5-4.0 wt% |
| Cu | 1.2-2.0 wt% |
| Co | 0.0-0.2 wt% |
| Al | 0.05-0.4 wt% |
| Ti | 1.9-2.3 wt% |
| Nb | 0.2-0.5 wt% |
| W | 0.0-0.6 wt% |
based on the alloy weight, the remaining being Fe, with Fe at least 30 wt%, and impurities, said impurities comprising S 0.0-0.001 wt% and P 0.0-0.02 wt%.

5. The component of claim 4, wherein the alloy has a chemical composition consisting of:
| | |
|---|---|
| C | 0.005-0.02 wt% |
| Si | 0.05-0.2 wt% |
| Mn | 0.1-0.6 wt% |
| Cr | 20.0-21.5 wt% |
| Ni | 35.0-37.0 wt% |
| Mo | 3.5-4.0 wt% |
| Cu | 1.2-2.0 wt% |
| Co | 0.0-0.2 wt% |
| Al | 0.05-0.4 wt% |
| Ti | 1.9-2.3 wt% |
| Nb | 0.2-0.5 wt% |
| W | 0.0-0.6 wt% |
based on the alloy weight, the remaining being Fe, with Fe at least 30 wt%, and impurities, said impurities comprising S 0.0-0.001 wt% and P 0.0-0.02 wt%.

6. The component of claim 5, wherein the alloy has a chemical composition consisting of:
| | |
|---|---|
| C | 0.005-0.02 wt% |
| Si | 0.06-0.15 wt% |
| Mn | 0.2-0.4 wt% |
| Cr | 20.2-21.0 wt% |
| Ni | 36.0-36.5 wt% |
| Mo | 3.6-3.8 wt% |
| Cu | 1.3-1.7 wt% |
| Co | 0.0-0.1 wt% |
| Al | 0.1-0.3 wt% |
| Ti | 2.0-2.2 wt% |
| Nb | 0.25-0.4 wt% |
| W | 0.0-0.4 wt% |
based on the alloy weight, the remaining being Fe, with Fe at least 30 wt%, and impurities, said impurities comprising S 0.0-0.001 wt% and P 0.0-0.015 wt%.

7. The component of claim 6, wherein the alloy has a chemical composition consisting of:
| | |
|---|---|
| C | 0.015 wt% |
| Si | 0.09 wt% |
| Mn | 0.3 wt% |
| Cr | 20.4 wt% |
| Ni | 36.2 wt% |
| Mo | 3.7 wt% |
| Cu | 1.41 wt% |
| Co | 0.03 wt% |
| Al | 0.25 wt% |
| Ti | 2.04 wt% |
| Nb | 0.27 wt% |
| W | 0.1 wt% |
| Fe | balance |
having the following impurities:
| | |
|---|---|
| P | up to 0.013 wt% |
| S | up to 0.0002 wt% |
| B | up to 0.003 wt% |
| Bi | up to 0.3 ppm |
| Ca | up to 50 ppm |
| Mg | up to 30 ppm |
| Ag | up to 5 ppm |
| Pb | up to 5 ppm |
| N | up to 100 ppm |
| Sn | up to 50 ppm |
| O | up to 50 ppm |

8. A process for making the component made of the alloy of any one of claims 1-7, said process comprising at least one of the following steps of:
a) melting the chemical composition of any one of claims 1-7 through vacuum induction melting (VIM), or arc electric furnace;
b) refining by Argon Oxygen Decarburization (A.O.D.), Vacuum Induction Degassing and Pouring (V.I.D.P), or Vacuum Oxygen Decarburization (V.O.D.);
c) re-melting through electro-slag re-melting (E.S.R.), or vacuum arc re-melting (VAR).

9. The process of claim 8, further comprising the step d) of homogenization of the alloy resulting from said at least one step, at a temperature above 1100° C for at least 6 hours.

10. The process of claim 9, further comprising a step e) of hot or cold plastic deformation through at least one plastic deformation cycle.

11. The process of claim 10, further comprising a step f) of heat treatment to induce solubilization through at least one heat cycle, at a temperature of 1020-1150°C, and followed by fast cooling in liquid or gas media.

12. The process of claim 11, further comprising a step g) of an ageing treatment.

13. The process of claim 12, wherein said step g) of an ageing treatment comprises the following sub-steps:
g-1) heating the alloy to a temperature of 710-780°C for 4-8 h;
g-2) cooling at a cooling rate of 40-60°C/h down to a temperature of 610-670°C;
g-3) keeping the alloy to a temperature of 610-670°C for at least 6 h, and
g-4) letting the alloy to cool at room temperature in air,
or comprises the following sub-steps:
g-1') heating the alloy to a temperature of 780-820°C for 2-8 h; and
g-2') letting the alloy to cool at room temperature in air.

14. The process of any one of claim 8-13, wherein the resulting alloy is further atomized to produce powder and then treated by powder metallurgy selected from Cold Isostatic Pressing (CIP), Metal Injection Moulding (MIM), Sintering, Hot Isostatic Pressing (HIP), or MIM and HIP process.

15. A turbomachine comprising at least one component according to any one of claims 1-7.

## Patentansprüche

1. Komponente einer Turbomaschine, wobei die Komponente hergestellt ist aus einer eine chemische Zusammensetzung aufweisenden Legierung, bestehend aus:
| | |
|---|---|
| C | 0,005-0,03 Gew.-% |
| Si | 0,05-0,5 Gew.-% |
| Mn | 0,1-1,0 Gew.-% |
| Cr | 19,5-22,5 Gew.-% |
| Ni | 35,0- 37,0 Gew.-% |
| Mo | 3,0-5,0 Gew.-% |
| Cu | 1,0-2,0 Gew.-% |
| Co | 0,0-1,0 Gew.-% |
| Al | 0,01-0,5 Gew.-% |
| Ti | 1,8-2,5 Gew.-% |
| Nb | 0,2-1,0 Gew.-% |
| W | 0,0- 1,0 Gew.-% |
bezogen auf das Legierungsgewicht, wobei das Verbleibende Fe und Verunreinigungen sind, wobei die Verunreinigungen 0,0-0,01 Gew.-% S und 0,0-0,025 Gew.-% P umfassen.

2. Komponente nach Anspruch 1, wobei die Legierung eine hohe Korrosionsbeständigkeit bei einer hohen Temperatur, speziell in dem Bereich von 200-250°C, aufweist.

3. Komponente nach Anspruch 1 oder 2, wobei die Legierung eine hohe Beständigkeit gegenüber Ermüdung und/oder Kriechen bei einer hohen Temperatur, speziell in dem Bereich von 400-700°C, aufweist.

4. Komponente nach einem der Ansprüche 1-3, wobei die Legierung eine chemische Zusammensetzung aufweist, bestehend aus:
| | |
|---|---|
| C | 0,005-0,03 Gew.-% |
| Si | 0,05-0,2 Gew.-% |
| Mn | 0,1 -0,6 Gew.-% |
| Cr | 20,0-21,5 Gew.-% |
| Ni | 35,0-37,0 Gew.-% |
| Mo | 3,5-4,0 Gew.-% |
| Cu | 1,2-2,0 Gew.-% |
| Co | 0,0-0,2 Gew.-% |
| Al | 0,05-0,4 Gew.-% |
| Ti | 1,9-2,3 Gew.-% |
| Nb | 0,2-0,5 Gew.-% |
| W | 0,0-0,6 Gew.-% |
bezogen auf das Legierungsgewicht, wobei das Verbleibende Fe mit mindestens 30 Gew.-% Fe und Verunreinigungen ist, wobei die Verunreinigungen 0,0-0,001 Gew.-% S und 0,0-0,02 Gew.-% P umfassen.

5. Komponente nach Anspruch 4, wobei die Legierung eine chemische Zusammensetzung aufweist, bestehend aus:
| | |
|---|---|
| C | 0,005-0,02 Gew.-% |
| Si | 0,05-0,2 Gew.-% |
| Mn | 0,1-0,6 Gew.-% |
| Cr | 20,0-21,5 Gew.-% |
| Ni | 35,0-37,0 Gew.-% |
| Mo | 3,5 -4,0 Gew.-% |
| Cu | 1,2-2,0 Gew.-% |
| Co | 0,0-0,2 Gew.-% |
| Al | 0,05-0,4 Gew.-% |
| Ti | 1,9-2,3 Gew.-% |
| Nb | 0,2-0,5 Gew.-% |
| W | 0,0-0,6 Gew.-%, |
bezogen auf das Legierungsgewicht, wobei das Verbleibende Fe mit mindestens 30 Gew.-% Fe und Verunreinigungen ist, wobei die Verunreinigungen 0,0-0,001 Gew.-% S und 0,0-0,02 Gew.-% P umfassen.

6. Komponente nach Anspruch 5, wobei die Legierung eine chemische Zusammensetzung aufweist, die besteht aus:
| | |
|---|---|
| C | 0,005-0,02 Gew.-% |
| Si | 0,06-0,15 Gew.-% |
| Mn | 0,2-0,4 Gew.-% |
| Cr | 20,2-21,0 Gew.-% |
| Ni | 36,0-36,5 Gew.-% |
| Mo | 3,6-3,8 Gew.-% |
| Cu | 1,3-1,7 Gew.-% |
| Co | 0,0-0,1 Gew.-% |
| Al | 0,1-0,3 Gew.-% |
| Ti | 2,0-2,2 Gew.-% |
| Nb | 0,25-0,4 Gew.-% |
| W | 0,0-0,4 Gew.-%, |
wobei das Verbleibende Fe mit mindestens 30 Gew.-% Fe und Verunreinigungen ist, wobei die Verunreinigungen 0,0-0,001 Gew.-% S und 0,0-0,015 Gew.-% P umfassen.

7. Komponente nach Anspruch 6, wobei die Legierung eine chemische Zusammensetzung aufweist, bestehend aus:
| | |
|---|---|
| C | 0,015 Gew.-% |
| Si | 0,09 Gew.-% |
| Mn | 0,3 Gew.-% |
| Cr | 20,4 Gew.-% |
| Ni | 36,2 Gew.-% |
| Mo | 3,7 Gew.-% |
| Cu | 1,41 Gew.-% |
| Co | 0,03 Gew.-% |
| Al | 0,25 Gew.-% |
| Ti | 2,04 Gew.-% |
| Nb | 0,27 Gew.-% |
| W | 0,1 Gew.-%, |
| Fe | Rest |
mit den folgenden Verunreinigungen:
| | |
|---|---|
| P | bis zu 0,013 Gew.-% |
| S | bis zu 0,0002 Gew.-% |
| B | bis zu 0,003 Gew.-% |
| Bi | bis zu 0,3 ppm |
| Ca | bis zu 50 ppm |
| Mg | bis 30 ppm |
| Ag | bis 5 ppm |
| Pb | bis 5 ppm |
| N | bis 100 ppm |
| Sn | bis 50 ppm |
| O | bis 50 ppm |

8. Verfahren zum Herstellen der Komponente, die hergestellt ist aus der Legierung nach einem der Ansprüche 1-7, wobei das Verfahren mindestens einen der folgenden Schritte umfasst:
a) Schmelzen der chemischen Zusammensetzung nach einem der Ansprüche 1-7 durch Vakuuminduktionsschmelzen (VIM) oder Lichtbogenelektroofen;
b) Raffinieren mittels Argon-Sauerstoff-Entkohlung (A.O.D.), Vakuum-Induktionsentgasen und Gießen (V.I.D.P) oder Vakuum-Sauerstoff- Entkohlung (V.O.D.);
c) Umschmelzen durch Elektroschlacke-Umschmelzen (E.S.R.) oder Vakuum-Lichtbogen-Umschmelzen (VAR).

9. Verfahren nach Anspruch 8, weiter umfassend den Schritt d) der Homogenisierung der Legierung, die aus dem mindestens einen Schritt resultiert, bei einer Temperatur oberhalb von 1.100°C für mindestens 6 Stunden.

10. Verfahren nach Anspruch 9, weiter umfassend einen Schritt e) der heißen oder kalten plastischen Verformung durch mindestens einen plastischen Verformungszyklus.

11. Verfahren nach Anspruch 10, weiter umfassend einen Schritt f) der Wärmebehandlung zum Einleiten einer Solubilisierung durch mindestens einen Wärmezyklus bei einer Temperatur von 1.020-1.150°C und gefolgt von schnellem Abkühlen in flüssigen oder gasförmigen Medien.

12. Verfahren nach Anspruch 11, weiter umfassend einen Schritt g) einer Alterungsbehandlung.

13. Verfahren nach Anspruch 12, wobei der Schritt g) einer Alterungsbehandlung die folgenden Unterschritte umfasst:
g-1) Erhitzen der Legierung bis zu einer Temperatur von 710-780°C für 4-8 h;
g-2) Kühlen bei einer Kühlgeschwindigkeit von 40-60°C/h bis zu einer Temperatur von 610-670°C;
g-3) Halten der Legierung auf einer Temperatur von 610-670°C für mindestens 6 h, und
g-4) Kühlenlassen der Legierung bei Raumtemperatur in Luft,
oder die folgenden Unterschritte umfasst:
g-1') Erhitzen der Legierung bis zu einer Temperatur von 780-820°C für 2-8 h; und
g-2') Kühlenlassen der Legierung bei Raumtemperatur in Luft.

14. Verfahren nach einem der Ansprüche 8-13, wobei die resultierende Legierung weiter zerstäubt wird, um Pulver zu erzeugen, und danach mit Hilfe von Pulvermetallurgie behandelt wird, ausgewählt aus kaltisostatischem Pressen (CIP), Metallspritzgießen (MIM), Sintern, heißisostatischem Pressen (HIP) oder MIM- und HIP-Verfahren.

15. Turbomaschine, umfassend mindestens eine Komponente nach einem der Ansprüche 1-7.

## Revendications

1. Composant d'une turbomachine, le composant étant fait d'un alliage ayant une composition chimique consistant en :
| | |
|---|---|
| C | 0,005 à 0,03 % en poids |
| Si | 0,05 à 0,5 % en poids |
| Mn | 0,1 à 1,0 % en poids |
| Cr | 19,5 à 22,5 % en poids |
| Ni | 35,0 à 37,0 % en poids |
| Mo | 3,0 à 5,0 % en poids |
| Cu | 1,0 à 2,0 % en poids |
| Co | 0,0 à 1,0 % en poids |
| Al | 0,01 à 0,5 % en poids |
| Ti | 1,8 à 2,5 % en poids |
| Nb | 0,2 à 1,0 % en poids |
| W | 0,0 à 1,0 % en poids |
sur la base du poids de l'alliage, le reste étant Fe et des impuretés, lesdites impuretés comprenant 0,0 à 0,01 % en poids de S et 0,0 à 0,025 % en poids de P.

2. Composant selon la revendication 1, dans lequel l'alliage présente une résistance élevée à la corrosion à température élevée, en particulier dans la plage allant de 200 à 250 °C.

3. Composant selon la revendication 1 ou 2, dans lequel l'alliage présente une résistance élevée à la fatigue et/ou au fluage à température élevée, en particulier dans la plage allant de 400 à 700 °C.

4. Composant selon l'une quelconque des revendications 1 à 3, dans lequel l'alliage présente une composition chimique consistant en :
| | |
|---|---|
| C | 0,005 à 0,03 % en poids |
| Si | 0,05 à 0,2 % en poids |
| Mn | 0,1 à 0,6 % en poids |
| Cr | 20,0 à 21,5 % en poids |
| Ni | 35,0 à 37,0 % en poids |
| Mo | 3,5 à 4,0 % en poids |
| Cu | 1,2 à 2,0 % en poids |
| Co | 0,0 à 0,2 % en poids |
| Al | 0,05 à 0,4 % en poids |
| Ti | 1,9 à 2,3 % en poids |
| Nb | 0,2 à 0,5 % en poids |
| W | 0,0 à 0,6 % en poids |
sur la base du poids de l'alliage, le reste étant Fe, avec au moins 30 % en poids de Fe, et des impuretés, lesdites impuretés comprenant 0,0 à 0,001 % en poids de S et 0,0 à 0,02 % en poids de P.

5. Composant selon la revendication 4, dans lequel l'alliage présente une composition chimique consistant en :
| | |
|---|---|
| C | 0,005 à 0,02 % en poids |
| Si | 0,05 à 0,2 % en poids |
| Mn | 0,1 à 0,6 % en poids |
| Cr | 20,0 à 21,5 % en poids |
| Ni | 35,0 à 37,0 % en poids |
| Mo | 3,5 à 4,0 % en poids |
| Cu | 1,2 à 2,0 % en poids |
| Co | 0,0 à 0,2 % en poids |
| Al | 0,05 à 0,4 % en poids |
| Ti | 1,9 à 2,3 % en poids |
| Nb | 0,2 à 0,5 % en poids |
| W | 0,0 à 0,6 % en poids |
sur la base du poids de l'alliage, le reste étant Fe, avec au moins 30 % en poids de Fe, et des impuretés, lesdites impuretés comprenant 0,0 à 0,001 % en poids de S et 0,0 à 0,02 % en poids de P.

6. Composant selon la revendication 5, dans lequel l'alliage présente une composition chimique consistant en :
| | |
|---|---|
| C | 0,005 à 0,02 % en poids |
| Si | 0,06 à 0,15 % en poids |
| Mn | 0,2 à 0,4 % en poids |
| Cr | 20,2 à 21,0 % en poids |
| Ni | 36,0 à 36,5 % en poids |
| Mo | 3,6 à 3,8 % en poids |
| Cu | 1,3 à 1,7 % en poids |
| Co | 0,0 à 0,1 % en poids |
| Al | 0,1 à 0,3 % en poids |
| Ti | 2,0 à 2,2 % en poids |
| Nb | 0,25 à 0,4 % en poids |
| W | 0,0 à 0,4 % en poids |
sur la base du poids de l'alliage, le reste étant Fe, avec au moins 30 % en poids de Fe, et des impuretés, lesdites impuretés comprenant 0,0 à 0,001 % en poids de S et 0,0 à 0,015 % en poids de P.

7. Composant selon la revendication 6, dans lequel l'alliage présente une composition chimique consistant en :
| | |
|---|---|
| C | 0,015 % en poids |
| Si | 0,09 % en poids |
| Mn | 0,3 % en poids |
| Cr | 20,4 % en poids |
| Ni | 36,2 % en poids |
| Mo | 3,7 % en poids |
| Cu | 1,41 % en poids |
| Co | 0,03 % en poids |
| Al | 0,25 % en poids |
| Ti | 2,04 % en poids |
| Nb | 0,27 % en poids |
| W | 0,1 % en poids |
| Fe | le reste |
ayant les impuretés suivantes :
| | |
|---|---|
| P | jusqu'à 0,013 % en poids |
| S | jusqu'à 0,0002 % en poids |
| B | jusqu'à 0,003 % en poids |
| Bi | jusqu'à 0,3 ppm |
| Ca | jusqu'à 50 ppm |
| Mg | jusqu'à 30 ppm |
| Ag | jusqu'à 5 ppm |
| Pb | jusqu'à 5 ppm |
| N | jusqu'à 100 ppm |
| Sn | jusqu'à 50 ppm |
| O | jusqu'à 50 ppm. |

8. Procédé de fabrication du composant fait de l'alliage selon l'une quelconque des revendications 1 à 7, ledit procédé comprenant au moins l'une des étapes suivantes :
a) la fusion de la composition chimique selon l'une quelconque des revendications 1 à 7 par fusion sous vide par induction (VIM), ou dans un four électrique à arc ;
b) un affinage par décarburation à l'argon-oxygène (A.O.D.), par dégazage et coulée sous vide par induction (V.I.D.P), ou par décarburation sous vide par l'oxygène (V.O.D.);
c) une refusion par refusion sous laitier électroconducteur (E.S.R.), ou par refusion à l'arc sous vide (VAR).

9. Procédé selon la revendication 8, comprenant en outre l'étape d) d'homogénéisation de l'alliage résultant de ladite au moins une étape, à une température supérieure à 1100 °C pendant au moins 6 heures.

10. Procédé selon la revendication 9, comprenant en outre une étape e) de déformation plastique à chaud ou à froid dans au moins un cycle de déformation plastique.

11. Procédé selon la revendication 10, comprenant en outre une étape f) de traitement thermique pour induire une solubilisation dans au moins un cycle de traitement thermique, à une température de 1020 à 1 150°C, et suivie d'un refroidissement rapide dans un milieu liquide ou gazeux.

12. Procédé selon la revendication 11, comprenant en outre une étape g) de traitement de vieillissement.

13. Procédé selon la revendication 12, dans lequel ladite étape g) de traitement de vieillissement comprend les sous-étapes suivantes :
g-1) le chauffage de l'alliage à une température de 710 à 780 °C pendant 4 à 8 heures ;
g-2) un refroidissement à une vitesse de refroidissement de 40 à 60°C/heure jusqu'à une température de 610 à 670 °C ;
g-3) le maintien de l'alliage à une température de 610 à 670 °C pendant au moins 6 heures, et
g-4) le fait de laisser l'alliage refroidir à température ambiante à l'air,
ou comprend les sous-étapes suivantes :
g-1') le chauffage de l'alliage à une température de 780 à 820 °C pendant 2 à 8 heures ; et
g-2') le fait de laisser l'alliage refroidir à température ambiante à l'air.

14. Procédé selon l'une quelconque des revendications 8 à 13, dans lequel l'alliage résultant est en outre atomisé pour produire une poudre et ensuite traité par une métallurgie des poudres sélectionnée parmi la compression isostatique à froid (CIP), le moulage par injection de poudre métallique (MIM), le frittage, la compression isostatique à chaud (HIP), ou un procédé MIM et HIP.

15. Turbomachine comprenant au moins un composant selon l'une quelconque des revendications 1 à 7.
